

# UNITED STATES PATENT OFFICE.

JACQUES DELPECH, OF PARIS, FRANCE.

## PROCESS OF MANUFACTURING GUN-POWDERS.

1,316,360.

Specification of Letters Patent. Patented Sept. 16, 1919.

No Drawing.

Application filed April 29, 1918. Serial No. 293,529.

To all whom it may concern:

Be it known that I, JACQUES DELPECH, citizen of the Republic of France, and resident of Paris, France, (post-office address 5 19 Avenue Parmentier,) have invented a new and useful Process of Manufacturing Gun-Powders, which improvements are fully set forth in the following specification.

The present invention relates to the manufacture of powder. With increase of artillery power the progressive action of propulsive powder becomes from day to day a feature of greater importance, with the object of diminishing the maximum pressure 10 or enabling certain ballistic problems to be solved without exceeding the pressure limit compatible with the weapon used. This increase in the progressive action has up to now been attempted with partial success by 15 shaping the grains of the powder in such a way that the surface provided for the emission of gas instead of diminishing, tends to increase as combustion proceeds.

Other attempts have been made on other 20 lines, which may be termed chemical. Here the object in view is to diminish the power and the brisance of the powder, when it starts to burn, by superficial gelatinization, varnishing or similar processes; however, 25 these processes only partially attain their end. They are unsuitable for powders intended for use in heavy artillery and generally speaking these attempts have proved to be of little practical use, while at the same 30 time, they are troublesome to carry out.

The problem has now been solved by forming heterogeneous powders in which there is a central core of a more brisant and powerful character surrounded by a layer 35 or sheet of powder which is less brisant and less powerful. In practice the following method is adopted:—

A sheet of the more brisant powder which is obtained by ordinary means of manufacture is inclosed between two sheets or layers of less brisant powder. After having united 40 the three (or more) of these layers of powder together (by the means hereinafter described) the resulting thick sheet is cut in 45 the usual manner to the desired dimensions (disks, pellets, tablets, strips and the like). It has been found that perfect adhesion can be obtained between the covering layers and the middle or core layer, by exterior pressure 50 in the cold or warm either by means of a hydraulic press or by passing the three or

more sheets of powder through suitably arranged rollers. In such case the union may be facilitated by coating one or more of the sheets with a substance which acts as solvent 60 for the powder.

The chemical composition and the thickness of the superimposed sheets of the core may be altered within very wide limits and allow the action (i. e., the commencement of 65 combustion) of the central core to be controlled so that it takes place at the most suitable point in the bore of the weapon. Furthermore, the fact that the combustion starts with a less brisant powder considerably lessens 70 wear and tear of the weapon as has been shown by the most recent researches of various investigators.

Finally powders with a central core coated with one or more superimposed layers of 75 colloidal powder of a different composition from that of the central core shows indisputable advantages from the point of view of progressive action and the lessening of the wear and tear of the weapon in which 80 they are used.

What I claim and desire to secure by Letters Patent of the United States is:—

1. The process for the production of powder consisting in disposing an interior sheet of 85 brisant colloidal powder between exterior sheets of less brisant colloidal powder said sheets being caused to adhere by any suitable mechanical pressure, the sheets being afterward cut into the desired shapes and dimensions. 90

2. The process for the production of powder consisting in disposing an interior sheet of brisant colloidal powder containing nitro-glycerin between exterior sheets of less 95 brisant colloidal powder said sheets being caused to adhere by any suitable mechanical pressure, the sheets being afterward cut into the desired shapes and dimensions.

3. The process for the production of 100 powder consisting in disposing an interior sheet of brisant colloidal powder containing nitro-glycerin between exterior sheets of less brisant colloidal powder also containing nitro-glycerin said sheets being caused to adhere by any suitable mechanical pressure, the sheets being afterward cut into the desired shapes and dimensions. 105

4. The process for the production of powder consisting in disposing an interior 110 sheet of brisant colloidal powder between exterior sheets of less brisant colloidal powder

said sheets being caused to adhere by passing them through cylindrical rollers, the sheets being afterward cut into the desired shapes and dimensions.

5. 5. The process for the production of powder consisting in disposing an interior sheet of brisant colloidal powder between exterior sheets of less brisant colloidal powder said sheets being caused to adhere by pressing them in a hydraulic press, the sheets being afterward cut into the desired shapes and dimensions.

10. 6. The process for the production of powder consisting in disposing an interior sheet of brisant colloidal powder containing nitro-glycerin between exterior sheets of less brisant colloidal powder containing nitro-glycerin said sheets being caused to adhere by passing them through cylindrical rollers, the sheets being afterward cut into the desired shapes and dimensions.

15. 7. The process for the production of powder consisting in disposing an interior sheet of brisant colloidal powder between exterior sheets of less brisant colloidal powder, coating certain of said sheets with a solvent for the powder said sheets being

caused to adhere by any suitable mechanical pressure, the sheets being afterward cut into the desired shapes and dimensions. 30

8. The process for the production of powder consisting in disposing an interior sheet of brisant colloidal powder between exterior sheets of less brisant colloidal powder, coating certain of said sheets with a solvent 35 for the powder said sheets being caused to adhere by subjecting them to hydraulic pressure, the sheets being afterward cut into the desired shapes and dimensions.

9. The process for the production of 40 powder consisting in disposing an interior sheet of brisant colloidal powder between exterior sheets of less brisant colloidal powder said sheets being caused to adhere by any suitable pressure in the warm, the sheets being 45 afterward cut into the desired shapes and dimensions.

10. A powder comprising a core sheet of brisant powder inclosed between sheets of less brisant powder. 50

In testimony whereof I have signed this specification.

JACQUES DELPECH.